# EUROPEAN PATENT SPECIFICATION

(11) **EP 1 129 789 B1**
(45) Date of publication and mention of the grant of the patent: **21.06.2006**
(21) Application number: 00200746.6
(22) Date of filing: 03.03.2000
(51) Int. Cl.: B05D 7/14, B05D 7/22, B05D 5/08, F28F 19/04

(54) **Protection of the water-side surfaces of heat exchangers used in boilers and gas fired water heaters**
Oberflächenschutz der Wasserseiteoberfläche von Wärmeaustauscher von Heizkesseln und Gaswasserheizern
Protection des surfaces coté eau d'échangeurs de chaleur de chaudières et de chauffe-eau à gaz

(43) Date of publication of application: 05.09.2001
(73) Proprietor: Riello S.p.A., 37045 Legnago (IT)
(72) Inventor: Pastorino, Giorgio, Ing., 23864 Malgrate, Lecco (IT)
(74) Representative: Jorio, Paolo

(56) References cited:
- WO-A-92/16310
- WO-A-96/21836
- FR-A- 2 476 145
- GB-A- 2 084 486
- US-A- 4 082 140
- US-A- 4 125 152
- US-A- 4 344 993
- US-A- 4 503 099
- US-A- 4 588 643
- US-A- 5 562 156
- PATENT ABSTRACTS OF JAPAN vol. 010, no. 353 (M-539), 28 November 1986 (1986-11-28) & JP 61 149794 A (NISSAN MOTOR CO LTD), 8 July 1986 (1986-07-08)

## Description

### 1. State of Art

All heat exchangers producing hot water, are subject to limestone precipitation of calcium and magnesium carbonates and to fouling of the circuits due to residual working products or other foreign matters present in the water network.

Besides, in case water contains some particular additives (for instance glycoles), the migration of metallic ions (Copper, Aluminium, Stainless Steel) may occur. The corrosion of metallic surfaces is always potentially possible.

The precipitation of limestone is more significant, the higher is the water limestone contents (hardness of water), the higher is the water heating and the longer is the time water remains at high temperature.

The fouling due to limestone and solid foreign matters present in the network occurs in different types of exchangers, such as:
- Bi-thermic exchangers for the combined production of hot water both for ambient heating and for sanitary (Fig. 1).
- Primary exchangers for the production of hot water for ambient heating only (Fig. 2).
   - Plate-type exchangers for the production of sanitary hot water (Fig. 3).
   - Storage vessels for the production and the storage of sanitary hot water (Fig. 4).
   - Additional storage systems for sanitary hot water.
   - Exchangers for water heaters.

The exchangers intended for the production of sanitary hot water (plate-type, primary exchangers, vessels, sanitary water tanks and bi-thermic exchangers) shall keep drinkable the sanitary water produced according to WRC standards.

The metals used for exchangers are, according to the type:
Copper (Cu DHP, CU OF, SE CU)
Stainless Steel (AISI 316L, AISI 304)
Aluminium

The water-diluted product has a viscosity comparable to water viscosity and is such as to fill all the interstices of the exchangers.

The exchangers nowadays on sale need to be frequently cleaned with specific acids to remove limestone crusts and dirt deposits causing in the run of time the obstruction of the passages and the thermal unbalance of the exchangers.

JP 61-149 794 discloses a method wherein scale deposits are prevented by coating the inner surface of an heat exchanger with a layer containing a fluorosilicon resin, which is circulated in a freon solution; this method therefore requires use of a freon-diluted resin, which is complicated to be used.

### 2. Description of the invention

In order to limit the above undesired effects, a procedure has been developed to treat the exchange surfaces with particular fluorurated resins. Such resins are provided with functional groups that adhere to the metallic surfaces to create a few microns thick coating limiting the adhesion of limestone and of the deposits present in heating circuits.

The peculiar features of the treatment, i.e. the anti-adhesion of limestone on the coated surfaces, have been checked both at IABER S.p.A. test laboratory (Ann. 1) and at the laboratory of the resin Manufacturer (Ann. 2), and through tests "on the field".

The performance of the thermal exchange and the hydraulic characteristics of the exchangers are not at all modified by the treatment.

The resin coating treatment is performed as it is shown in the diagram of Fig. 5.

The water-diluted product has a viscosity comparable to water viscosity and such as to fill all the interstices of the exchangers.

### 3. Innovations introduced by the invention

The treatment of exchangers and vessels with fluorinated resins allows to overcome one of the weakest points of exchangers i.e. a reduced performance in the run of time due to the deposit of limestone and dirt present in the network. Specifically, thanks to this treatment, the circuits obstructions due to the effects of limestone and of a variety of residual working products are reduced and, therefore, the useful life of the same exchangers in compliance with specifications is extended.

Particularly, limestone keeps on precipitating during the water heating but, when precipitated, it does not adhere firmly to walls. On the contrary, it is eliminated by the same water stream. Similarly, thanks to the anti-adhering characteristics of the treatment, foreign matters in water (dirt and residual working products) do not fix to the exchangers walls but they slide away together with the water stream.

Moreover, the surface protection from such resins reduces the migration of metallic ions in water, the corrosion of the same metals and assures a higher water sanitation coming into contact with the water-side surfaces.

### 4. Patent Right Claims

The protection we claim with patent shall cover the application procedure of water-deluted fluorinated products with low viscosity on the metallic surfaces made of Copper (CU DHP, CU OF, SE CU), Aluminium and Stainless Steel (AISI 316L, AISI 304) of the heat exchangers and vessels used for the production of sanitary hot water and ambient heating in storage or instantaneous gas-fired wall boilers and in water heaters.

The effect of the treatment is:
1. to limit the limestone deposit;
2. to limit the deposit of residual working products;
3. to keep unaltered the sanitation characteristics of the produced sanitary water
4. to keep unaltered the thermal exchange characteristics. 5.

### 5. Laboratory tests carried out by IABER S.p.A.

Limestone tests have been carried out on treated vessels boiling the same quantity of water on a camp stove:
1. VESSEL No. 1 : Heat-treated Copper without special treatments
2. VESSEL No. 2 : Green Teflon SR43F coated Copper
3. VESSEL No. 3 : Ausimont Silane coated Copper

### REMARKS:

Limestone deposits occur in Vessels No. 1 and No. 2, which do not detach from the walls.

In Vessel No. 3 the limestone patina does not deposit on the walls and with the addition of fresh water the limestone solution dissolves.

### 6. Laboratory tests carried out on account of IABER S.p.A.

The coating with functional perfluorpolyetheric products has been laid on some copper plates, in compliance with ordinary procedures.

The product has been applied by dip-coating with the following treatment formulas:
1. 1-Phosphate
2. 5-Phosphate
3. 1-Silane
4. 5-Silane

Copper test specimen has been plunged into the compounds for 10 minutes before heat-treatment:
- Heating at T = 80°C for 7 minutes
- Heating at T = 65°C for 40 minutes
- Heating at T = 160°C for 12 minutes

Subsequent to the preparation of the specimen, some measurements of static and dynamic contact angle versus water, hexadecane, dodecane, decane and octane were carried out. Only the results relevant to the measurement of the static contact angle versus water carried out before limestone deposition, after deposition and after washing under cold tap water are herein reported.

### Contact angle measurements for treated/untreated copper specimen, before limestone deposition (table 1 shown in Fig. 6).

### Contact angle measurements for treated/untreated copper specimen, after limestone deposition:

A calcium bicarbonate solution has been prepared. This is more soluble in water than the calcium carbonate (limestone) that tends to form and deposit at temperatures higher than 50°C. The treated/untreated specimen have been plunged into these boiling solutions for 3 hours. At the end of this time, the limestone deposit on all specimen was recorded; on specimen treated with Silane, however, the amount of the deposit was the lowest (also on phosphate a certain effect was noted). Here below the measurements of static contact angle versus water after limestone deposition under the described conditions are recorded (table 2 shown in Fig. 7).

### Contact angle measurements for treated/untreated copper specimen, after washing under tap flowing water:

Test specimen have been washed under a stream of cold tap-water for few seconds; after this time specimen have been stove-dried for 15 minutes and then the static contact angle versus water was measured again (table 3 shown in Fig. 8).

The best treatment proved to be that with silanes (5-Silane specimen) showing:
- lower limestone deposit
- greater easiness in removing limestone
- lower copper oxidation

## Claims

1. A method for preventing precipitation of limestone and deposit of residual working products or other foreign matters on inner surfaces of heating circuits having metallic surfaces made of copper, stainless steel or aluminium, comprising the steps of:
- dissolving a silane fluorinated resin provided with functional groups to prepare a diluted product;
- filling the circuit to be processed with the diluted product;
- emptying the circuit;
the method being **characterized in that** said resin is dissolved in water thereby forming a water-diluted product having a viscosity comparable to water viscosity, and **in that** said functional groups of the resin are functional groups that adhere to said metallic surfaces made of copper, stainless steel or aluminium.

2. A method as claimed in claim 1, **characterized in that** said resin is a silane fluorinated resin provided with perfluoropolyetheric groups.

3. A method as claimed in claim 1 or 2, **characterized in that** said step of emptying the circuit is performed by flowing compressed air into the circuit.

4. A method as claimed in any of the preceding claims, **characterized by** comprising, after the step of emptying the circuit, the step of cooking said circuit in an oven.

## Patentansprüche

1. Verfahren zum Verhindern der Ablagerung von Kalk und dem Absetzen von Rest-Verarbeitungsprodukten oder anderen Fremdkörpern an inneren Oberflächen von Heizkreisläufen, die aus Kupfer, Edelstahl oder Aluminium erzeugte metallische Oberflächen aufweisen, umfassend die Schritte:
- Lösen eines fluorierten Silanharzes, das mit funktionellen Gruppen versehen ist, um ein gelöstes Produkt herzustellen;
- Befüllen des zu bearbeitenden Kreislaufs mit dem gelösten Produkt;
- Leeren des Kreislaufs;
wobei das Verfahren **dadurch gekennzeichnet ist, dass** das Harz in Wasser gelöst wird, wodurch ein wassergelöstes Produkt ausgebildet wird, das eine Viskosität aufweist, die mit der des Wassers vergleichbar ist, und dass die funktionellen Gruppen des Harzes funktionelle Gruppen sind, die an den aus Kupfer, Edelstahl oder Aluminium erzeugten metallischen Oberflächen anhaften.

2. Verfahren wie in Anspruch 1, **dadurch gekennzeichnet, dass** das Harz ein fluorierter Silanharz ist, das mit Perfluorpolyether-Gruppen versehen ist.

3. Verfahren wie in Anspruch 1 oder 2, **dadurch gekennzeichnet, dass** der Schritt des Leerens des Kreislaufs durch Einströmen komprimierter Luft in den Kreislauf durchgeführt wird.

4. Verfahren wie in einem der voranstehenden Ansprüche, **dadurch gekennzeichnet, dass** es nach dem Schritt des Leerens des Kreislaufs den Schritt des Erwärmens des Kreislaufs in einem Ofen umfasst.

## Revendications

1. Procédé pour empêcher la précipitation de tartre et le dépôt de produits actifs résiduels ou d'autres matières étrangères sur les surfaces intérieures de circuits de chauffage ayant des surfaces métalliques en cuivre, acier inoxydable ou aluminium, comprenant les étapes de :
- dissolution d'une résine fluorée de type silané comportant des groupes fonctionnels, pour préparer un produit dilué ;
- remplissage du circuit à traiter avec le produit dilué ;
- vidange du circuit ;
le procédé étant **caractérisé en ce que** la dite résine est dissoute dans l'eau afin de former un produit dilué dans l'eau ayant une viscosité comparable à la viscosité de l'eau, et **en ce que** les dits groupes fonctionnels de la résume sont des groupes fonctionnels qui adhèrent aux dites surfaces métalliques en cuivre, acier inoxydable ou aluminium.

2. Procédé selon la revendication 1, **caractérisé en ce que** la dite résine est une résine fluorée de type silarte comportant des groupes perfluoropolyéther.

3. Procédé selon la revendication 1 ou 2, **caractérisé en ce que** la dite étape de vidange du circuit est effectuée par circulation d'air comprimé dans le circuit.

4. Procédé selon une quelconque des revendications précédentes, **caractérisé en ce qu'**il comprend, après l'étape de vidange du circuit, l'étape de cuisson du dit circuit dans un four.
